

Patented Sept. 28, 1926.

1,601,541

# UNITED STATES PATENT OFFICE.

BY RAMJI D. SAKLATWALLA, OF CRAFTON, PENNSYLVANIA.

## MANUFACTURE OF CHROMIUM ALLOY STEEL.

No Drawing.

Application filed March 11, 1922. Serial No. 543,081.

The present invention relates to the manufacture of chromium alloy steel and more particularly to the reduction of the chromium directly from the ore and the production 5 of a low-carbon chromium alloy steel. A molten bath of steel is formed having a metal layer containing a carbonaceous reducing agent and a slag layer containing the unreduced chromium compound or ore 10 and a reaction takes place between the carbon in the metal layer and the unreduced chromium compound in the slag layer whereby metallic chromium is introduced directly into the steel.

15 In the manufacture of chromium steel, under the prevailing practice existing hitherto, the chromium content was generally introduced in the form of a ferro-alloy. As the regular commercial grades of ferro-chromium contain an appreciable percentage 20 of carbon, this practice introduced an undue amount of carbon in the steel. This is particularly objectionable in the so-called "stainless" steels or irons which have a high 25 chromium content, usually in the neighborhood of 9% to 15%, because the presence of carbon in such steels has a greater physical effect than the same amount of carbon in ordinary steel; for example 1/10 of 1% of 30 carbon in the high chromium stainless steel has about the same physical effects as 4/10% of carbon in the ordinary steel. A stainless iron should contain less than 1/10 of 1% of carbon.

35 It is not commercially practicable to de-carburize the steel after the addition of the carbon-containing ferro-chromium, because the processes of oxidizing the carbon are accompanied by an oxidation and consequent 40 waste of the valuable chromium content.

On the other hand, if special grades of low ferro-chromium are used, their cost is so high as to prohibitively increase the cost 45 of the steel produced. The defects or disadvantages in adding the commercial grades of ferro-chromium or the special grades of low-carbon ferro-chromium are particularly apparent in the manufacture of the so-called "stainless" steels or irons, where a large 50 quantity of ferro-chromium has to be added, since the percentage of chromium must be high, usually between 9% and 15% and the carbon content should be very low.

In accordance with the present invention, 55 the carbon content of the steel is greatly reduced by the addition of the chromium com-

pound or ore, and the chromium may be obtained from a source very much cheaper than ferro-chromium. The chromium is added preferably in the form of chrome or chromite to a bath of molten steel in any ordinary steel-making furnace, and chromium is reduced from the chromite by means of the carbon, and possibly other reducing agents present in the steel. By this means, 60 the chromium is introduced into the steel, and at the same time, the carbon content is eliminated or reduced to the desired minimum. The process may be carried out in the following manner:

65 Pig iron or pig iron and scrap are melted in an ordinary steel-making furnace, such as an open-hearth furnace. After the metal is molten, the requisite quantity of chrome ore, together with lime and fluorspar, as fluxes, is charged on top of the molten bath. When the reaction between the chromium oxide of the chromium ore and the carbon in the bath ceases, the metal is tapped. The lime and fluorspar added with the chrome ore as fluxes help to refine the 70 finished steel from impurities, such as sulphur and phosphorus. This refining can also be further controlled by increasing the furnace temperature before tapping. The fluorspar added with the lime makes a more liquid slag and is added because the alumina and magnesia in the chromite, although forming a basic slag, do not make a sufficiently liquid slag.

75 If a considerable proportion of chromium is to be added in the form of chrome ore, the amount of the reducing agent in the steel may be increased either by adding pig iron or other high carbon irons or steels, or by introducing another reducing agent, such as silicon or manganese, into the bath. The carbon exists in the pig iron or other high carbon irons or steels principally in the form of iron carbide. Silicon may be 80 added in the form of ferro-silicon, or may be in the form of a chrome silicon alloy. Such a chrome silicon alloy may be cheaply prepared and may contain in the neighborhood of 30% to 35% silicon, 40% chromium, and the remainder iron and impurities. The amount of chromite or chrome ore added should be in sufficient quantity to reduce the carbon or the carbon and silicon content to 85 the desired minimum. The slag will contain some chromium or chromite which will be wasted, but this is not a serious objection.

since the chromite ore is comparatively cheap.

The specifications for steel and iron are, in general, much more rigid on the tolerance limits for carbon and silicon than they are for chromium. It is therefore advantageous to add the chromite to the steel containing known quantities of carbon or carbon and silicon. The chromite may be 5 added in quantities regulated to reduce the carbon or carbon and silicon, and if analysis of the sample shows that the carbon or carbon and silicon are not sufficiently reduced, more chromite may be added, since the limits 10 of tolerance of the chromium generally vary over a few percent. In this way, a much more minute and accurate control of the carbon and silicon limits may be secured than would be the case if they were introduced into the steel at the same time as the chromite ore.

If desired, the carbon or silicon content may be slightly increased after the oxidizing reaction of the chromite ore takes place, 25 for example, as by the addition of a small amount of ferro-silicon to deoxidize the steel, and reduce a further amount of the chromium.

The process is intended principally as an 30 open-hearth or electric furnace process, although it may be used with a crucible or any other steel-making furnace.

The source of chromium and oxygen which causes the reaction to reduce the carbon or carbon and silicon and add chromium is preferably chromite on account of its cheapness, although other sources of chromium may be used.

The silicon if used may be added in the 40 form of ferro-silicon or chrome silicon alloy; and the term "silicon" as herein employed, is intended to cover various forms of silicon or silicon-bearing materials or alloys.

The term "steel" as herein employed is 45 intended as a term of general description and not of limitation, and is intended to include the so-called "stainless irons" which are, in reality, steels having a very low carbon and metalloid content. The term "chrome steel" is also intended as a term of general description and not of limitation, and is intended to include steels having chromium as the principal alloying metal, 50 although containing other alloying metals.

The tolerance limitation of the alloying metals and the metalloids in steels is very much closer than in the so-called ferro alloys, such for example, as ferrochromium, 60 and it is therefore necessary to carry out steel making processes under much more carefully regulated and controlled conditions than processes of making ferro alloys.

In carrying out my process the carbon, which is the major reducing agent, is present

in an amount which is predetermined by the chromium content of the steel. The process is not one of decarbonizing a metal bath having an unknown or fortuitous amount of carbon, but is a process of making a chrome 70 steel having the desired chromium content in which the amount of the carbonaceous reducing agent is predetermined and carefully regulated.

The carbon reducing agent may be incorporated into the molten metal of the bath by melting down a charge containing the requisite amount of carbon, or the carbonaceous reducing agent may be added later to the completed bath in regulated amounts, 75 preferably in the form of pig iron or other high carbon irons or steels which of course have a sufficient specific gravity to sink 80 through the slag layer and carry the carbon into the metal layer. An unreduced 85 chromium compound, such for example, as chromite, may be introduced into the slag layer at any suitable or convenient time, either during the melting down of the charge or after the bath is completely 90 formed. The specific gravity of these unreduced compounds is such that they will naturally gravitate to and become incorporated in the slag layer.

The reducing reaction apparently takes 95 place across the interface between the metal layer and the slag layer. The reduced chromium in its nascent state is in contact with the steel bath and therefore the best 100 conditions are obtained for the alloying of the reduced chromium and its dissemination throughout the steel.

While the preferred embodiment of the present invention has been specifically described, it is to be understood that the present invention is not limited to the herein described details and may be otherwise embodied in processes of making chromium alloy steel within the scope of the following 110 claims.

I claim:

1. Those steps in the process of making chrome steel, which comprise introducing the major portion, if not all, of the chromium into the steel by forming a molten bath of steel having a metal layer containing carbon as the major reducing agent in an amount predetermined by the desired chromium content of the steel and a slag layer in which is incorporated chrome ore and maintaining the bath in a molten condition so as to cause a reaction between the carbon in the metal layer and the chrome ore in the slag layer to thereby directly reduce chromium into the steel, substantially as 115 described.

2. Those steps in the process of making chrome steel, which comprise introducing the major portion, if not all, of the chromium into the steel by forming a molten bath 120

125

130

of steel having a metal layer and a slag layer, adding a carbide to the metal layer in an amount predetermined by the desired chromium content of the steel and adding 5 chrome ore to the slag layer, and maintaining the bath in a molten condition so as to cause a reaction between the carbide in the metal layer and the chrome ore in the slag layer to thereby directly introduce the reduced metallic chromium into the steel, substantially as described.

3. Those steps in the process of making chrome steel, which comprise forming a molten bath of steel having a metal layer 15 containing carbon as the principal reducing agent and a slag layer in which is incorporated an unreduced chromium compound, maintaining the bath in a molten condition so as to cause a reaction between the carbon in the metal layer and the unreduced chromium compound in the slag layer to thereby directly reduce the chromium into the steel, and thereafter increasing the 20 temperature of the bath to further refine the steel before tapping, substantially as described.

4. Those steps in the process of making chrome steel, which comprise introducing the major portion, if not all, of the chromium 30 into the steel by forming a molten bath of steel having a metal layer containing carbon as the major reducing agent in an amount

predetermined by the desired chromium content of the steel and a slag layer in which is incorporated chrome ore and a fluxing material which produces a slag with the gangue of the ore which removes objectionable metalloids from the steel and maintaining the bath in a molten condition so as to cause a reaction between the carbon and the ore to thereby directly reduce into the steel the 35 chromium from its ore simultaneously with the refining of the steel, substantially as described.

5. Those steps in the process of making chrome steel, which comprise introducing the major portion, if not all, of the chromium into the steel by forming a molten bath of steel having a metal layer containing carbon as the major reducing agent and a slag layer 50 in which is incorporated an unreduced chromium compound, maintaining the bath in a molten condition so as to cause a reaction between the carbon in the metal layer and the unreduced chromium compound in the slag layer to thereby directly reduce chromium into steel, and thereafter adding a silicon reducing agent to the steel to reduce 55 more of the chromium, substantially as described.

In testimony whereof I have hereunto set my hand.

BYRAMJI D. SAKLATWALLA.